

Jan. 22, 1946.

J. D. GOLD ET AL

2,393,363

HEAT TREATMENT OF THIN METAL ARTICLES

Filed March 15, 1943

3 Sheets-Sheet 1



Fig. 1

Inventors:  
J. D. Gold,  
C. D. Foulke,

James Stanley  
Attorney

Jan. 22, 1946.

J. D. GOLD ET AL

2,393,363

HEAT TREATMENT OF THIN METAL ARTICLES

Filed March 15, 1943

3 Sheets-Sheet 2



Fig. 2.



Fig. 3.

Fig. 4.

Inventors  
J.D. GOLD & C.D. FOULKE

By *James J. Sherry* attorney

Jan. 22, 1946.

J. D. GOLD ET AL

2,393,363

HEAT TREATMENT OF THIN METAL ARTICLES

Filed March 15, 1943

3 Sheets-Sheet 3



Fig. 5.



Fig. 6.



Fig. 7.



Fig. 8.

Inventors

J. D. GOLD & C. D. FOULKE

*James J. Slattery*  
Attorney

## UNITED STATES PATENT OFFICE

2,393,363

## HEAT TREATMENT OF THIN METAL ARTICLES

John D. Gold and Clarence D. Foulke, Steubenville, Ohio, assignors to National Steel Corporation, a corporation of Delaware

Application March 15, 1943, Serial No. 479,246

12 Claims. (Cl. 148—10)

The present invention relates to an improved process of producing thin metal articles having controlled temper and the product thereof.

In the cold working of metals the crystalline structure is modified so that the resulting product is extremely hard and in the case of sheet metal and wire very stiff. In order to adapt metals treated in this manner to use for certain products an annealing treatment is necessary which relieves the strains set up in the metal by the cold working and leaves the metal in soft condition. Other products require metal which is neither as hard as in the cold worked condition nor as soft as in the full annealed condition. Attempts have been made to arrive at an intermediate hardness or temper by partial or "work" annealing. Under annealing methods now in use it is extremely difficult if not impossible to arrive at an intermediate product with consistently controlled temper.

As an example of the problem involved and present practice, thin sheet steel called black plate for ultimate manufacture into tin plate is now commonly produced as a product of a continuous cold rolling step. A slab of low carbon steel is hot rolled down to about 16 gauge on a continuous hot strip mill. The hot rolled strip is passed through a continuous pickling line to remove the hot mill scale and is then passed through a continuous cold mill where it is reduced to black plate gauge, commonly between .025 and .005 of an inch in thickness. In the usual practice coils of this cold reduced strip, after the cold mill oil has been removed, are box annealed to dead soft condition. Since sheet steel in this condition is too soft for tin plate, temper must be imparted to it. This is normally done by passing the full soft strip through skin pass or temper mills where a very accurately controlled percentage of reduction gives the desired temper.

A specific example of the problem of arriving at the correct temper may be studied relative to tin plate to be used in can bodies. In such product the stiffer the tin plate the lighter the gauge sheet which may be used. The stiffness is limited however by the ability of the plate to form a side seam. If the plate will not produce a seam which remains flat, it is too stiff. On the other hand, if the plate is too soft, fluting will occur when the cylindrical body is being formed. A much stiffer tin plate is desired for can ends and bottle tops, but black plate in its full hard condition is too stiff for even these products.

The present invention is a process for produc-

ing thin sheet metal of desired temper. The product of the present process is an improved metal sheet. Although the term "temper" in the art of producing sheets and strip is usually applied to hardness or stiffness of the sheet or strip metal as developed by cold working, the term is used herein to designate hardness or stiffness of sheet or strip metal as arrived at by a special heat treatment of metal initially in cold worked condition. According to the present invention a full hard sheet metal or wire is heat treated under exacting conditions to result directly in a sheet of the desired hardness and stiffness herein called temper. To arrive at this product of controlled temper, the strained condition of the metal is relieved for only a portion of the thickness of the sheet or cross section of the wire. Thus the portion of the thickness in which strain is unrelieved supplies stiffness while the remaining portion modifies the over-all effect in the article. Strain is relieved at at least one surface of the sheet by recrystallization of the grain structure at and adjacent to that surface. It will be apparent that in making a bend which puts such surface in tension the greater ductility of the recrystallized and partially recrystallized metal will be beneficial, while the layer of uncryallized metal will furnish a stiffness to prevent fluting and supply rigidity to the sheet.

Although sheet and strip metal are specifically described herein, it will be obvious that metal in strand or wire form will respond as readily to the process. The same applies to metal in tubular or pipe form. The criterion in any case is the existence of an initially full hard metal article in a form having a small thickness dimension, so a desirable over-all stiffness of the article is effected by controlling recrystallization of the grain structure adjacent a surface while leaving a layer of unrelieved strained structure. As used in this description and in the appended claims the term "sheet metal" is intended to cover any such article of determinate length and the term "metal strip" is intended to cover any such article of indeterminate length including wire. The term "thin metal article" as used in this description and in the appended claims is intended to include the above two terms.

An important object of the present invention is the provision of a process for producing sheet metal or metal strip of controlled temper by a heat treatment of the metal in cold worked condition.

A further important object of the present invention is the provision of a method for produc-

ing sheet metal or metal strip of controlled temper from the full hard product by effecting varying degrees of recrystallization of the grain structure through the thickness of the sheet or strip.

A further important object of the present invention is the provision of a continuous process for producing a sheet metal or metal strip of controlled temper from the full hard product by heat treatment.

A further important object of the present invention is the provision of a process for controlling the temper of sheet metal or metal strip by utilizing the "skin effect" of high frequency induction heating.

A further important object of the present invention is the provision of an improved product of controlled temper resulting from the present heat treatment of full hard metal.

Other objects and advantages of this invention will become apparent from the following detailed description, reference being had to the accompanying drawings which constitute a part of this specification and wherein:

Figure 1 consists of reproductions enlarged to about  $1\frac{1}{4}$  of original size of actual photomicrographs at a magnification of 100 of steel treated in accordance with the present invention.

Figure 2 is a schematic showing of one form

ing of the surface of a metal article and since the small thickness dimension of the articles involved sometimes necessitates the equivalent of a quenching action to prevent undesirable penetration of the heat into the article, it will be obvious that the invention is limited in such cases to the treatment of those metals which are usually considered nonhardening by quenching methods. Thus the high carbon steels and special alloy hardening steels cannot be treated by the present invention where a quenching step is necessary.

In the case of steel, for example, sheets of full hard black plate of .0095" thickness were positioned with both surfaces in contact with heat supplying surfaces at a temperature of 1500° F. The samples of black plate were maintained in contact with these heat supplying surfaces for varying intervals of time to control closely the depth of heat penetration. The black plate was water quenched immediately following contact with the heat supplying surfaces. Photomicrographs of cross sections of the treated black plate showing varying degrees of recrystallization through the thickness appear in Figure 1. Tests show the physical properties for the treated specimens as set out in Table I below, the untreated black plate shown at "a" in Figure 1 being full hard with a Rockwell 30-T of 81.

Table I

|                                      | Figure                      |                             |                  |                  |
|--------------------------------------|-----------------------------|-----------------------------|------------------|------------------|
|                                      | 1b                          | 1c                          | 1d               | 1e               |
| Time of heat application.....seconds | 1 $\frac{1}{4}$             | 2 $\frac{1}{4}$             | 3 $\frac{1}{4}$  | 4 $\frac{1}{4}$  |
| Rockwell 30-T.....                   | 76                          | 73                          | 68               | 66               |
| Can forming.....                     | No fluting                  | No fluting                  | No fluting       | No fluting       |
| Side seam.....                       | Will not seam<br>180° flat. | Will not seam<br>180° flat. | Seams 180° flat. | Seams 180° flat. |

of apparatus for continuously carrying out the process of the present invention.

Figure 3 is a schematic showing of another form of apparatus for continuously carrying out the process of the present invention.

Figure 4 is a schematic view of apparatus for continuously carrying out a second embodiment of the process of the present invention.

Figure 5 is a schematic showing of apparatus for continuously carrying out the process of the present invention utilizing high frequency induction heating currents.

Figure 6 is a schematic showing of a cross section through a coil adapted to be used in the apparatus of Figure 5, and

Figures 7 and 8 are views representing photomicrographs of a cross section through articles treated in accordance with the process of the present invention.

In the present process an external surface of the cold worked article is subjected to a temperature great enough to raise this surface above a critical value. When this surface reaches this critical value, recrystallization of the grain structure is initiated. This recrystallization is allowed to proceed until a depth of recrystallized grain structure is arrived at which in the finished article, acting in conjunction with the remaining unrelieved material, will give the desired over-all temper or physical characteristics. The temperature of that section of the article in which recrystallization is occurring is then reduced to inhibit further recrystallization and further penetration of the heat into the unrelieved section. Since the present invention involves softening

Obviously by raising the temperature of the heat supplying surfaces within limits, shorter contact time would be necessary.

From Table I it will be apparent that the specimen shown at "d" in Figure 1 would be highly suitable for can bodies.

The remnants of the chilled and free freezing crystals from the ingot may under some conditions influence the results. Such influence is of a favorable nature since the free freezing crystals occur in the intermediate section of the thickness of the article and therefore retard recrystallization in this section relative to the rate of recrystallization in the sections adjacent the surface where the chilled crystals exist.

In order to treat strip metal continuously in accordance with the present process, apparatus of the type shown in Figure 2 may be utilized. The strip metal 10 being fed from a coil of cold reduced metal is passed into an insulated furnace structure 11, wherein it passes between two heated rolls 12. The strip passes from between the rolls out of furnace 11 and into immediate contact with two cooling rolls 13. The temperature of heated rolls 12 is such that the heat supplied to the surface of the strip is sufficient to initiate recrystallization and carry on the same through the thickness of the strip by heat penetration. Cooling rolls 13 are positioned relative to heating rolls 12 so that with the strip moving at the desired speed, heat is abstracted from the surfaces of the strip to prevent further recrystallization and penetration of the heat. A controlled depth of recrystallized grain structure is thus achieved, leaving an intermediate layer of unrelieved

lieved grain structure. Since the time of contact between strip and the heated rolls and the cooling rolls is limited, the speed of the strip must be limited.

With the apparatus shown in Figure 3 a higher strip speed can be attained, the strip being maintained in contact longer with the heating and cooling rolls. With this apparatus the strip 10 enters an insulated furnace 14 and makes prolonged contact with heating roll 15. The strip is then immediately contacted in the same manner with cooling roll 16. The other side of the strip is next contacted with hot roll 17 followed by cold roll 18. Here again the temperature of the heating rolls and the speed of the strip are so related that the desired degree of recrystallization part way through the strip is accomplished before the cooling rolls abstract sufficient heat to stop recrystallization.

In Figure 4 an apparatus is shown for carrying out an embodiment of the present invention wherein only one surface of a strip is treated. A strip 19 enters an insulated furnace structure 20 and is guided by idler roller 21 onto the surface of a heating roll 22. The strip leaves the heating roll and passes into contact with a cooling roll 23. An idler roller 24 guides the treated strip to a recoiling or further treating station (not shown). Strip produced in the apparatus of Figure 4 will have the metal at one surface in strained and unrelieved condition while at the other surface the metal will be in relieved condition with the grain structure completely to partially recrystallized.

The hot rolls are formed of heat resistant material having a smooth surface to avoid marring the strip. The cooling rolls are formed with copper surfaces or some such material having good heat conductivity. Heat may be supplied to the hot rolls by an internal flame, hot fluid, electrical heating elements or in any desired manner.

The apparatus schematically shown in Figure 5 includes an insulated furnace structure 25 having therein a high frequency electromagnetic induction coil 26. A strip 27 passes into furnace 25 through induction coil 26 out of furnace 25 into a quenching zone 28 and thence to further handling. In the process employed with the apparatus of Figure 5 a high frequency voltage is applied to coil 26. The voltage is such that in view of the frequency, sufficient heat is supplied to the strip by induced currents to effect the desired degree of recrystallization. The frequency is so designed that the skin effect confines the induced currents in proximity to the surfaces of the strip. The disposition of the induced currents in this manner can thus be used to supply heat only at the points where recrystallization of grain structure is desired. Strip metal of magnetic nature is most favorably treated in this manner.

Prompt abstraction of the heat following passage of the strip through the coil inhibits further recrystallization, but this may not be necessary if the heat supplied is not excessive. Although a liquid bath 29 is shown, any desirable form of quenching or cooling means may be used when this step is desired. The desired frequency must be arrived at by experimentation for each shape of article being treated. A frequency in the neighborhood of one megacycle will produce sufficient skin effect to successfully treat 98# black plate in accordance with the present invention.

Where flat strip material is being treated an induction coil surrounding the strip will not give the proper distribution of heat unless it is prop-

erly shaped. The edges of the strip will receive energy from both the sides and the ends of the coil. In Figure 6, strip 30 is shown passing through a coil 31 designed to eliminate unequal distribution of energy to the strip. Where desired the shape of the coil as in Figure 6 may be such that some sections of the sheet receive more energy than the others. Since segregation tends to be more prevalent in one section of a strip such as the center, giving a greater annealing effect at such a section may result in a product having more uniform characteristics across its width.

Obviously, where wire is being treated, a cylindrical coil will be effective.

In order to prevent oxidation of the material an inert atmosphere may be desired. In the apparatus of Figures 2 to 4 inclusive, means 32 is shown for introducing inert gas into a casing 33 enclosing the cooling rolls. Sealing means 34 at the strip exit point force the gas to circulate into the furnace and out at the strip entrance point. In the case of the apparatus of Figure 5, the gas is introduced by means 35 directly into the furnace.

Where desired or necessary sufficient tension is maintained on the strip to prevent objectionable buckling of the hot strip.

Figure 7 shows a cross section of a product produced by the process carried out in the apparatus of Figure 4. In this case it is apparent that the recrystallization is initiated from only one side of the article, the material at the other surface being in unrelieved condition. This will result in a sheet having better bend characteristics in one direction than the other due to the material adjacent one surface being of much greater ductility.

Figure 8 shows a cross section of wire treated in accordance with the present invention in the apparatus of Figure 5. The article having been cold drawn has a grain orientation in the direction of the length. A section taken through the center of the wire of Figure 8 along the length will have the same appearance as the showing in Figure 1b to Figure 1f depending on the degree of treatment desired.

When the article being treated is wire it will be apparent that a product of high tensile strength and great flexibility will result. The core of the wire being in full hard unrelieved condition will have a high tensile strength while the outer annealed portions will form a jacket of soft ductile material.

The heat can be imparted to the strip or wire for the present process by any of the well known heating baths such as molten salt baths.

We claim:

1. A process for softening a thin, elongated ferrous metal article which is in cold work hardened condition comprising raising the temperature of an elongated surface of the article sufficiently to initiate recrystallization adjacent the surface and controlling the temper of the product by controlling the heat penetration into the article to prevent complete recrystallization throughout the thickness of the article.

2. A process for softening a thin, elongated ferrous metal article which is in cold work hardened condition comprising supplying heat at an elongated surface of the article to effect recrystallization adjacent the surface and controlling the temper of the product by controlling penetration of the heat through the thickness of

the article to effect a decreasing degree of recrystallization from the surface inwardly.

3. A process for treating a thin, elongated ferrous metal article which is in cold rolled condition, the article being formed of a ferrous metal substantially nonhardening by quenching methods, the steps comprising passing an elongated surface of the article into contact with a heat supplying medium to initiate recrystallization adjacent the surface and passing the article into contact with a cooling medium to control the heat penetration into the article to prevent complete recrystallization throughout the thickness of the article to thereby control the temper of the product.

4. A process of softening cold drawn, work hardened, elongated wire of ferrous metal comprising supplying heat at an elongated surface of the wire to effect recrystallization adjacent the surface and controlling the temper of the product by controlling the heat penetration into the wire to give a decreasing degree of recrystallization toward the center of the wire.

5. A process for treating a thin, elongated ferrous metal article which is in cold worked condition, the article being formed of a ferrous metal substantially nonhardening by quenching methods, the steps comprising setting up a high frequency electromagnetic field in the article to induce heating currents therein, the frequency of the field being such that skin effect confines the major portion of the currents adjacent the elongated surface of the article, supplying sufficient heat with the currents to initiate recrystallization at the elongated surface and controlling the temper of the product by controlling heat penetration into the article to prevent complete recrystallization throughout the thickness of the article.

6. A process for treating a thin, elongated ferrous metal article which is in cold worked condition, the article being formed of a ferrous metal substantially nonhardening by quenching methods, the steps comprising passing the article through an alternating electromagnetic field having a frequency such that heating currents are induced at the elongated surface of the article and withdrawing the article from the field when recrystallization has been effected adjacent the elongated surface and before heat penetration can

50 effect recrystallization throughout the thickness of the article to thereby control the temper of the product.

7. A process for treating a thin, elongated ferrous metal strip which is in cold worked condition, the strip being formed of a ferrous metal substantially nonhardening by quenching methods, the steps comprising passing the strip through an alternating electromagnetic field having a frequency such that heating currents are induced at the elongated surface of the strip, withdrawing the strip from the field when recrystallization has been effected adjacent the elongated surface and before heat penetration can effect recrystallization throughout the thickness of the sheet, and passing the strip through a quenching zone to abstract heat from the surface to thereby arrive at a controlled temper in the product.

8. A process for treating an elongated ferrous metal sheet or strip which is in cold worked condition, the sheet or strip being formed of a ferrous metal substantially nonhardening by quenching methods, the steps comprising supplying heat at one of the elongated surfaces of the sheet or strip to effect recrystallization adjacent that surface and controlling the temper of the product by controlling penetration of the heat through the thickness of the sheet or strip to prevent recrystallization adjacent the other surface of the sheet or strip.

9. A thin ferrous metal article of controlled temper produced by the process of claim 1.

10. A thin ferrous metal article of controlled temper produced by the process of claim 2.

11. A thin ferrous metal article of controlled temper produced by the process of claim 8.

12. A thin, elongated ferrous metal article of controlled temper formed from a metal substantially nonhardening by quenching methods, the article being characterized by having a portion of its cross-section in strained condition as a result of a cold working operation and a portion of its cross-section adjacent an elongated surface in relieved condition as a result of a heat treatment, the extent of the portion in relieved condition determining the temper of the article.

JOHN D. GOLD.  
CLARENCE D. FOULKE.